

Patented Dec. 28, 1926.

1,612,570

# UNITED STATES PATENT OFFICE.

LEON CAMMEN, OF NEW YORK, N. Y.

MAKING IRON ALLOYS.

No Drawing.

Application filed March 26, 1926. Serial No. 97,774.

The present invention refers to a process for producing extremely low carbon steels, with special reference to so-called electric sheets, such as silicon steel sheets, and describes a process whereby an extremely low-carbon material may be obtained commercially.

T. D. Yensen (Transactions, American Institute of Electrical Engineers, vol. 34, pp. 10 2601 ff.) reports that by melting electrolytic iron alloyed with silicon in a vacuum furnace he has obtained a maximum permeability some 500 per cent higher than is encountered in commercial silicon steel sheets. While 15 this has been generally ascribed to the use of vacuum melting, my own work would indicate that the remarkable results obtained by Yensen were due primarily to the nearly total absence of carbon in his samples due to 20 the use of electrolytic iron as a starting material, and to the comparative freedom of the product from oxides and nitrides. In the present invention it is proposed to attain the same end by means that would permit to produce the desired material in 25 commercial quantities, at a price not too much above that of similar steels as now made. The process involves several stages.

The first stage is carried on in a Bessemer converter which is "overblown", i. e., blown until the iron begins to burn. This happens when both the silicon and the carbon blow are completed, and the blast still continued. At the end of such a blow the metal contains 30 a fairly low amount of carbon, say 0.05, and is heavily oxidized. It is then ready for the second stage which is carried on in some kind of a furnace which must satisfy two essential conditions: the furnace should be capable 35 to raise the temperature of the metal to 1550 deg. cent. or over, and there must be no chance for the metal to be contaminated by carbon (either solid as from the electrodes, or gaseous, as from carbon monoxide in the furnace atmosphere). An electric induction furnace satisfies these conditions.

At a temperature of the order of 1550 deg. cent., the tendency is for the carbon to 40 deoxidize iron. It is important however to bear in mind that the desired end is to reduce the carbon to say 0.001 per cent, and this means that even at 0.002 per cent the reaction of deoxidation of the iron oxide by carbon, 45 with consequent elimination of the carbon as

carbon monoxide, must continue. But 0.002 per cent carbon means 2 parts of carbon to 100,000 parts of the mass, or an extremely tenuous dilution, and of course no carbon-iron oxide reaction can take place unless the 50 carbon, or more precisely carbide of iron, come into direct contact with oxide of iron. Because of the extremely low content of carbon towards the end of the reaction, it is absolutely necessary that the oxide of iron, 55 while not in such quantities as to make its reduction to iron prohibitively expensive, should be so thoroughly distributed through the mass of the metal as to ensure in a positive manner the ability of every tiny drop of 60 carbide of iron to come into direct contact with a drop of oxide of iron.

It has been found that addition of iron ore to a metal bath does not insure such an intimate mixture of the oxide of iron 65 and the bath as to produce the desired result. It is for this reason that an "overblown converter stage" is used as the first stage, as it naturally results in an iron thoroughly and uniformly deoxidized, and such 70 handling as is necessary to transfer the metal from the converter to the induction furnace provides a stirring of the metal and increases its uniformity.

The time period during which the metal 75 has to be held in the induction furnace depends on several factors, such as the amount of decarbonization achieved in the Bessemer stage, and is a matter which any skilled metallurgist is capable of determining for 80 himself with due regard to the conditions of operation in his plant.

The metal is next deoxidized in the usual manner, and the proper additions of alloying elements, such as silicon, aluminum or 85 the like are made. In this part of the process common practice may be used.

This may be followed by the addition of such elements as zirconium, to eliminate sulfur, or titanium, to eliminate at least some 90 of the nitrogen or nitrides formed thereby.

The metal may be delivered to the furnace from the converter with the slag formed in the latter, and held in the furnace with this slag until the desired degree 95 of carbon reduction has been obtained, whereupon the converter slag is removed, and a deoxidizing slag is substituted.

Where conditions permit, a material increase in efficiency of the process may be se- 100

cured by operating the Bessemer stage in a somewhat unusual manner. In this case, the iron is supplied to the converter very hot, 1550 deg. cent. or over. When iron is blown 5 at this temperature, the carbon starts to burn before the silicon. At first the temperature is raised still more by the burning of the carbon, but as the amount of this latter decreases, the temperature falls off and finally 10 goes below the critical point for this process. When this happens, the silicon begins to burn, and by the time this is burnt out, the metal is reheated again to the temperature where it is capable of burning carbon. The 15 blowing should be however continued for a while even after the end of the second carbon-burning stage, so as to produce a very thorough distribution of oxides in the iron for the furnace stage.

20 Where manganese is used as deoxidizer, and the purpose is to produce a material of high magnetic permeability, the following variation of the process may be used. The second stage is carried out in a furnace with 25 a neutral bottom, the metal then being transferred into another similar furnace (which need not be run at such a high temperature) with an acid bottom. The advantage of using in this case an acid bottom lies in the 30 fact that silicon dioxide in the slag oxidizes the manganese in the metal, with the result that the silicon in the metal increases and manganese in the metal decreases, with simultaneous formation of MnO in the slag.

35 Low manganese in electric steel has been found to be an advantage. It is not always advisable to use an acid bottom, however, which is the reason for using here two electric furnaces: if the metal from the converter were delivered direct to an acid lined furnace and kept at the high temperature required here, there would be an intensive fluxing of the lining of the furnace, and its 40 life would be very short indeed. This does

not happen in the second furnace, as it receives the metal already fully deoxidized. 45

Where the term "furnace" is used in the claims, a furnace is meant such as defined in paragraph third on the first page of this specification, unless otherwise stated. 50

I claim:

1. A process of manufacture of iron alloys containing less than 0.03 per cent carbon by weight, comprising the following stages: first, the Bessemer stage wherein the blowing is continued until and beyond the end of the period of carbon burning; second, the furnace stage wherein the metal is held under such conditions that it cannot be contaminated by carbon, and a temperature is 60 maintained of the order of 1550 deg. cent. or more. 55

2. A process as described in claim 1, wherein the metal is delivered to the furnace from the converter with the slag 65 formed in the latter, and held in the furnace with this slag until the desired degree of carbon reduction has been attained, whereupon the converter slag is removed, and a deoxidizing slag is substituted. 70

3. A process as described in claim 1, wherein after the desired degree of carbon reduction has been attained, manganese is one of the deoxidizing elements added to the bath, and wherein the carbon reduction is 75 carried out in a furnace with a neutral lining, and the manganese deoxidation reaction substantially in a furnace with an acid lining.

4. A process as described in claim 1, 80 wherein the metal is delivered to the Bessemer converter at such a temperature that the carbon begins to burn ahead of the silicon.

Signed in New York, in the county and 85 State of New York, March 25, A. D. 1926.

LEON CAMMEN.